# EUROPEAN PATENT APPLICATION

(11) **EP 0 377 243 A1**
(43) Date of publication of application: **11.07.1990**
(21) Application number: 89203272.3
(22) Date of filing: 20.12.1989
(51) Int. Cl.: D02G 3/04, D03D 15/12

(54) **Flame-retardant textile structures with improved mechanical properties**

(30) Priority: 24.12.1988 NL 8803167
(71) Applicant: DSM N.V., 6411 TE Heerlen (NL)
(72) Inventor: Kriele, Johannes Elizabeth Adrianus, NL-4645 JJ Putte (NL)

(57) **Abstract**

Textile structures, treated with a flame-retardant, with improved wear-resistance and greater tear-resistance are obtained when the textile structures contain 3-30, preferably 5-15, wt.% polyalkylene fibres with a tensile strength of at least 2 GPa and a modulus of at least 60 GPa.

The flammability of the textile structures does not appear to have been substantially adversely affected by the inclusion therein of polyalkylene fibres.

## Description

The invention relates to textile structures that contain natural and/or man-made fibres and that have been treated with a flame-retardant.

Applications of such textile structures include, for example, the manufacture of fireproof clothing, or more fire-resistant curtains, upholstery fabric, floor covering, etc.

It has been found that textile structures that have been treated with flame-retardants and that contain natural and/or man-made fibres are less wear-resistant and less tear-resistant than untreated structures. The cause of these disadvantages could be the fact that solids precipitated from the flame-retardant have become attached to the fibres where they have an abrasive effect on the surrounding fibres. However, the disadvantage could also be partly due to the fact that the flame-retardant attacks the fibres chemically.

The aim of the invention is to provide textile structures containing natural and/or man-made fibres and having been treated with a flame-retardant, which textile structures show the aforementioned disadvantages in a greatly reduced degree and whose flame-retardant behaviour has not been adversely affected to any great extent.

This is achieved because the textile structures contain 3-30, preferably 5-15 wt.% polyalkylene fibres with a modulus of at least 60 GPa and a tensile strength of at least 2 GPa.

The textile structures according to the invention are clearly more wear-resistant and more tear-resistant than textile structures that do not incorporate polyalkylene fibres. The flammability of the textile structures does not appear to have been adversely affected to any great extent by the incorporation of polyalkylene fibres.

The incorporation of polyalkylene fibres in the textile structures to be treated with flame-retardants, for the purpose of improving the wear-resistance and the strength properties of the textile structure, presents the advantages, as compared with the use of other fibres with a high modulus and tensile strength such as fibres obtained from an aramide or poly-vinyl alcohol, that polyalkylenes have a lower density, are more resistant to ultra-violet radiation and absorb less moisture than the aforementioned other fibres. These advantages become very apparent when the textile structures are used for working clothes. The lower weight means greater comfort in wearing, the greater resistance to UV radiation does not only prevent discolouration but together with the low moisture-sensitivity it ensures that the textile structures maintain the desired properties with respect to wear-resistance and tear-resistance. It is surprising and unforeseeable that there are no substantial negative differences as regards flammability between textile structures treated with flame-retardants which include the indicated amounts of polyalkylene fibres and the same structures without said fibres.

Polyalkylene filaments with a modulus of at least 60 GPa and a tensile strength of at least 2 GPa that are used in the present invention can be obtained with the aid of a gel spinning process as described in GB-A-2.042.414 and GB-A-2.051.667. This process essentially consists in preparing a solution of a polyalkylene with a high weight average molecular weight (Mw > 4 x 10⁵), shaping the solution into filaments at a temperature above the dissolution temperature of the polymer, cooling the filaments to below the dissolution temperature to cause gelation and stretching the filaments and simultaneously removing the solvent.

Good results are obtained if polyethylene (PE) is chosen as polyalkylene. This PE may contain a small amount, preferably at most 5 mol.%, of one or more copolymerisable other alkylenes such as propylene, butylene, pentene, hexene, 4-methylpentene and octene and may have between 1 and 10, preferably 2-6 methyl or ethyl groups per 1000 carbon atoms.

Other polyolefins may also be used, for example polypropylene homo- and copolymers. In addition, the polyolefins used may contain small amounts of one or more other polymers, in particular alkene-1 polymers.

The polyalkylene filaments obtained according to the gel spinning process, with a modulus of at least 60 GPa and a tensile strength of at least 2 GPa, can be cut into staple fibres with lengths of 10 to 100 mm, preferably with lengths of 30-50 mm, and then be mixed with one or more fibres to a polyalkylene fibre content of 3-30 wt.%, preferably 5-15 wt.%. The other fibres may be natural, artificial or synthetic fibres or combinations thereof.

Natural fibres are here understood to be naturally occurring fibres such as cotton, wool, silk, jute, linen, etc. Artificial fibres are here understood to be fibres prepared from natural polymers, whether or not modified, such as rayon, which is prepared from cellulose. Synthetic fibres are here understood to be fibres that are prepared from a synthetic polymer such as polyamide fibres and polyester fibres.

A yarn is spun from the fibre mixture with the aid of the known suitable methods.

It is also possible to combine a yarn obtained from one or more fibres with polyalkylene filaments with a modulus of at least 60 GPa and a tensile strength of at least 2 GPa by means of for example twisting or core spinning.

The yarn is processed into a textile structure, for example a weave or a knit, with the aid of known suitable methods.

It is also possible to prepare a textile structure from different yarns, one of which contains a higher percentage of or consists entirely of fibres with a modulus of at least 60 GPa and a tensile strength of at least 2 GPa, and another of which contains a significantly lower percentage of such fibres or consists entirely of one or more other fibres. In this case, however, it is necessary that the textile structure thus obtained contains between 3 and 30 wt.%, preferably between 5 and 15 wt.% of polyalkylene fibres with a modulus of at least 60 GPa and a tensile strength of at least 2 GPa.

The textile structure is treated to reduce its flammability. A frequently applied treatment is impregnation with a solution or an emulsion of a flame-retarding product, followed by compression and drying. A possibility is, for example, impregnation with a solution of ammonium bromide. However, a textile structure treated with this agent looses its flame-retardant properties after washing. If a washable finish is required, a possibility is impregnation with a mixture of products that can react chemically with one another. For example, it is possible to use a mixture of tetrakis (hydroxymethyl)phosphonium chloride (THPC) with urea and trimethylolamide or a mixture of N-methylol-(dialkylphosphoniumpropionamide) with urea and trimethylolamide for impregnation. In this case after-heating is added to the treatment.

It may be preferable to treat the yarns spun from a mixture of 3-30, preferably 5-15 wt.%, polyalkylene fibres with a modulus of at least 60 GPa and a tensile strength of at least 2 GPa in order to reduce their flammability and to then process the thus treated yarns into a textile structure, which, if so desired, may also incorporate a small amount of some untreated yarn.

A textile structure, such as a fabric, that has been treated to reduce its flammability is excellently suitable for the manufacture of, for example, fireproof clothing such as overalls and for the manufacture of curtain and upholstery fabrics, floor covering, etc.

The invention will be elucidated below with the aid of a number of examples.

### Example 1

With the aid of a 3-cylinder cotton spinning machine the following yarns were spun, each having yarn number Ne 20/1:
yarn 1: 90 wt.% carded cotton fibres, 10 wt.% polyethylene fibres (Dyneema SK 60, TM), 1 denier, fibre length 40 mm. The polyethylene fibres have a tensile strength of 2.6 GPa and a modulus of 87 GPa.
yarn 2: 100% carded cotton fibres.
yarn 3: 90 wt.% carded cotton fibres, 10 wt.% polyester fibres (Terylene, TM), 1.5 denier, fibre length 40 mm.
yarn 4: 65 wt.% carded cotton fibres, 35 wt.% polyester fibres (Terylene, TM), 1.5 denier, fibre length 40 mm.
yarn 5: 90 wt.% carded cotton fibres, 10% aramide fibres (Keylar 29, TM), fibre length 40 mm.

A portion of each yarn was treated with a mixture of N-methylol(dialkylphosphoniumpropionamide), urea and trimethylolamide, produced by Ciba Geigy under the trade name Pyrovatex PC. The treatment was carried out according to the accompanying instructions, with the exception that the after-heating was done at a temperature of 130¤C instead of 150¤C.

The tensile strength was determined of the untreated and the treated impregnated yarns. The results are given in Table 1.

The results show, among other matters, that the treated yarns have a lower tensile strength than the untreated ones and that the yarns containing 10 wt.% polyethylene fibres or 35 wt.% polyester fibres have the highest tensile strength. It was also found that the yarn containing 10 wt.% polyethylene fibres shows a higher tensile strength than the yarn containing 10 wt.% aramide fibres.

**Table 1**

| Yarn | Tensile strength [N/Tex] | |
|---|---|---|
| | Untreated | Treated |
| 1 | 20.2 | 14.6 |
| 2 | 14.5 | 10.2 |
| 3 | 15.0 | 10.6 |
| 4 | 20.6 | 15.2 |
| 5 | 18.5 | 12.7 |

### Example 2

The untreated yarns 1, 2, 4 and 5 according to example 1 were used to produce fabrics A, B, C and D with a surface weight of 250 g/m² and a 4.1 satin weave.

The fabrics were treated with Pyrovatex PC (TM) as described in example 1. Fabric strips of 0.50 x 0.015 m were then subjected to burning tests according to DIN. 54336. The results are shown in Table 2.

The results show, among other matters, that the flammability of the treated fabric containing 10 wt.% polyethylene fibres is more or less the same as that of the treated fabric consisting entirely of cotton fibres. It was also found that a treated fabric containing 35% polyester fibres shows very unfavourable flammability.

**Table 2**

| Fabric | Ignition time | Burning time | Glowing time | Affected length |
|---|---|---|---|---|
| | (sec) | (sec) | (sec) | (mm) |
| A | 3 | 0 | 0 | 5 |
| A | 15 | 0 | 0 | 30 |
| B | 3 | 0 | 0 | 5 |
| B | 15 | 0 | 0 | 25 |
| C | 3 | burns | burns | 450 mm |
| C | 3 | burns | burns | 450 mm |
| D | 3 | 0 | 0 | 5 |
| D | 15 | 0 | 0 | 25 |

### Example 3

Fabrics A and D were subjected to intensive radiation for 100 hours in a Xenontester Hanau 1200 (TM). After 100 hours the colour of fabric A had not changed visibly whereas fabric D had clearly become darker.

### Example 4

The untreated yarns 1 and 2 according to example 1 were used to produce webs E and F, respectively, with a surface weight of 250 g/m² and a 4.1 satin weave, with a length of 0.5 m and a width of 0.05 m.

The fabrics were treated with Pyrovatex PC (TM) as described in example 1.

The fabrics were fixed in an abrasion test meter according to AATCC of the Crockmeter type. One side of the fabrics was clamped into the meter and a weight of 0.5 kg was attached to the other side to create the desired tension in the fabric.

The Crockmeter incorporates an abrasive block with an area of 0.05 * 0.03 m, provided with abrasive cloth with a fineness of grain of 220. The block was placed on the fabrics and was charged with a normal force of 0.1 kg.

The abrasive block was moved back and forth at an amplitude of 0.1 m. 1000 abrasion cycles were run at a frequency of 1 Hz. Before and after the test the tensile strengths of the fabrics were determined according to the usual method. The retention of strength of the fabrics is given in Table 3.

Table 3 shows that fabric E is less sensitive to wear.

## Claims

1. Textile structures that contain natural and/or synthetic fibres and that have been treated with a flame-retardant, characterized in that the textile structures contain 3-30 wt.% polyalkylene fibres with a modulus of at least 60 GPa and a tensile strength of at least 2 GPa.

2. Textile structures according to claim 1, characterized in that they contain 5-15 wt.% polyalkylene fibres with a modulus of at least 60 GPa and a tensile strength of at least 2 GPa.

3. Textile structures according to claim 1 or 2, characterized in that the poyalkylene fibre is a polyethylene fibre.

4. Textile structures according to any one of claims 1-3, characterized in that they contain cotton fibres.

5. Textile structures according to any one of claims 1-3, characterized in that the textile structures consist of cotton and polyethylene fibres.

6. Textile structures according to any one of claims 1-5, characterized in that they are made from yarns.

7. Textile structures according to any one of claims 1-5, characterized in that they are made from one type of yarn.

8. Textile structure according to claim 7, characterized in that the yarn consists of staple fibres.

9. Yarns that contain natural or synthetic fibres and that have been treated with a flame-retardant, characterized in that they contain a composition like that of the textile structures described in any one of claims 1-5.

10. Clothing, curtains, upholstery fabric and floor covering manufactured from textile structures according to any one of claims 1-8 or from yarns according to claim 9.
